

1

3,184,408  
HIGH TEMPERATURE STABILIZING  
LUBRICANT ADDITIVE

Ernest V. Wilson and Harry W. Rudel, Roselle, N.J.,  
assignors to Esso Research and Engineering Company,  
a corporation of Delaware  
No Drawing. Filed Dec. 14, 1961, Ser. No. 159,457  
5 Claims. (Cl. 252—32.7)

The present invention relates to compounded lubricating oils that are stabilized against thermal degradation and high temperatures. More particularly the invention concerns the use of additives that prevent the thermal decomposition of metal dialkyldithiophosphates in lubricating oil compositions under high temperature conditions.

It is well known to employ metal dialkyldithiophosphates in lubricating oil compositions for the purpose of improving the load carrying ability of the composition and to prevent wear. Normally, the use of such additives presents no serious problems when the concentration of the metal dialkyldithiophosphate is relatively low; i.e., in the range of about 0.1 to 0.5 wt. percent. It has recently been found however that, when it is necessary to increase the concentration of the additive to 1.0 wt. percent or more in certain compositions, there is a tendency for the metal dialkyldithiophosphates to decompose at high temperatures, causing the formation of heavy sediment and a strong odor and thus rendering the oil composition useless. This problem has arisen particularly in the case of marine turbine oils wherein cadmium salts of dialkyldithiophosphoric acids are employed to impart sufficient load carrying capacity to enable the oil to meet certain gear tests.

In order for a marine turbine oil to meet the specifications of the U.S. and Canadian Navies, its neutralization number must not exceed 0.2. It is possible to formulate a turbine oil meeting this specification which will, at the same time, have sufficient load carrying ability to pass certain gear tests by incorporating into the composition a cadmium dialkyldithiophosphate. Preferably, the dialkyldithiophosphates are derived from secondary alcohols averaging at least about 4.5 carbon atoms per alkyl group and preferably from about 6 to 12 carbon atoms per alkyl group. Secondary alcohols having from 3 to about 20 and preferably from about 3 to 13 carbon atoms may be used in the preparation of these additives. Lubricating oil compositions containing up to about 3 wt. percent of a cadmium dialkyldithiophosphate of the type described will have an ASTM D-974 neutralization number below 0.2. Lubricating oil compositions containing above about 1 to 1.25 wt. percent of this type of cadmium dialkyldithiophosphate will carry in excess of 3000 pounds in the Ryder gear test described in Military Specification MIL-L-17331B (Ships) 4.6.2.

Use of the cadmium dialkyldithiophosphate in this range of concentrations will also enable oil compositions to meet the IAE Gear Test requirement for specifications of both the British Navy (OEP-90) and the Canadian Navy (3GP-358T) as well as the FZG Gear Test (Niemann Test) requirements for merchant fleet acceptance in Germany.

Other metals such as lead and nickel will also give low neutralization numbers of the order of 4 or 5 when employed in a lubricating oil composition as compared with a neutralization number of about 180 in the case of the conventionally used antiwear agent zinc dialkyldithiophosphate.

While, as stated, it is possible to employ cadmium, nickel or lead dialkyldithiophosphate in lubricating oil compositions requiring high load carrying capacity and relatively low neutralization numbers, such compositions are limited in high temperature stability and tend to decompose ther-

2

mally under high temperature conditions such as exist in the Staeger oxidation test. The metal dialkyldithiophosphates tend to decompose and form sludge under such conditions.

5 In accordance with the present invention, it has been found that lubricating oil blends containing metal dialkyldithiophosphates can be effectively stabilized against thermal decomposition by incorporating therein a monoester of a trialkylolalkane of from about 6 to 12 carbon atoms and of a carboxylic acid selected from the group consisting of saturated and unsaturated fatty acids of from 12 to 20 carbon atoms and alkyl mercaptoacetic acids having alkyl groups of from about 9 to 18 carbon atoms. The monoesters that may be employed include those of trimethylolpropane, triethylolpropane and trimethylolbutane. The monoesters employed in the present invention are characterized by a neo structure. Specific examples are: trimethylolpropane monooleate, trimethylolpropane monostearate, triethylolpropane monosterate, triethylolbutane monolaurate, trimethylolpropane monopalmitate, and trimethylolpropane mono laurylmercaptopacetate.

10 The invention is particularly applicable to a marine turbine oil formulation containing a cadmium dialkyldithiophosphate in conjunction with a corrosion inhibitor of the type containing free carboxy groups. Corrosion inhibitors that have been found to be particularly useful in marine turbine oil formulations include mercaptoacetic acids having the formula: R—S—CH<sub>2</sub>—COOH, wherein R is a branched alkyl group containing in the range of 9 to 17 carbon atoms. Preferably R is a branched alkyl group of about 13 carbon atoms. Such branched chain alkyl groups may be derived from the well-known oxo alcohols which are prepared by reaction of olefins with carbon monoxide and hydrogen in the presence of a cobalt 15 or similar catalyst to form aldehydes of one more carbon atom than the starting olefins, followed by catalytic hydrogenation to the corresponding alcohols.

15 Also useful as rust inhibitors in the compositions of this invention are the alkenyl succinic acids having the following general formula:



20 45 wherein R represents an unsaturated aliphatic radical having about 10 to 22, preferably about 12 to 18 carbon atoms. Compounds wherein R is saturated are similarly useful. Rust inhibitors of this type are well known to the art and are described in U.S. Patents, e.g., 2,124,628 and 2,133,734. In practice the R group is generally a mixture of varying chain length averaging about C<sub>14</sub> to C<sub>18</sub>. Such compositions are preferred rust inhibitors for use in the lubricating oil compositions of this invention. The succinic acid or mercaptoacetic acid type rust inhibitors are used in concentrations in the range of 0.01 to 0.10 weight percent based on the total weight of the lubricating composition. Preferably, the concentrations of succinic acid type rust inhibitor are in the range of 0.03 to 0.05 weight percent of the total composition. Other rust inhibitors which may be used include dinonyl naphthalene sulfonates as described in U.S. Patent 2,764,548.

25 50 55 60 The dialkyldithiophosphoric acid salts of this invention are normally prepared by reacting the secondary alcohol or alcohol mixture containing a secondary alcohol with phosphorus pentasulfide



and then forming the cadmium salt by direct neutralization with cadmium oxide



Alternatively they may be prepared by double decomposition, e.g., by the reaction of an aqueous solution of an inorganic cadmium salt with an alkali metal dialkyldithiophosphate to form the corresponding lead or cadmium dialkyldithiophosphate. Regardless of the route of preparation, it is desired that the product have a low neutralization number and a composition corresponding closely to the theoretical values. The cadmium salt is normally prepared by direct neutralization of the acid with cadmium oxide (although good additives have been prepared by double decomposition).

The acid preparation involves the reaction of stoichiometric amounts of alcohol and phosphorus pentasulfide at a temperature in the range of 160 to 200° F., e.g., 185 to 190° F., for about 1 to 6 hours, e.g., about 3 hours. The acid will generally be filtered. The neutralization of the acid with CdO will be carried out at a temperature in the range of about 80 to about 200° F., e.g. 120 to 170° F. and will continue until the product is essentially neutral, about 1 to 6 hours, e.g., about 3 to 4 hours. It is understood that the temperatures and particularly the time of reaction will vary somewhat because of such factors as the size of the reaction mixture, the equipment being used, and so on. The product will usually be diluted with mineral oil or other suitable solvent to form a concentrate more easily handled than the pure additive.

While satisfactory products have been prepared under a variety of conditions within the ranges set forth above, for most consistent production of a satisfactory additive certain additional steps are taken. These are: (1) the phosphorus content of the  $\text{P}_2\text{S}_5$  is kept under the theoretical value of 27.87 wt. percent, preferably below about 27.8, e.g., 26.0-27.5; (2) the acid is blown free of  $\text{H}_2\text{S}$  with an inert gas, e.g., nitrogen, before neutralization; (3) elemental sulfur is added to the acid immediately before the neutralization. The last item, (3) above, is not always necessary if the  $\text{P}_2\text{S}_5$  used in the acid preparation has a phosphorus content toward the lower end of the range given in step (1) above. Of these precautionary steps, (1) appears most important.

The lubricating oils constituting the base stocks in the compositions of this invention are preferably mineral lubricating oils although synthetic oils may be used. Preferably the oil base has a viscosity in the range of 37 to 150 Saybolt seconds Universal at 210° F., a viscosity index in the range of 50 to 150, a flash point above 370° F., a pour point below 25° F. and a gravity in the range of 26 to 34° API. For turbine oil use a solvent neutral type of oil having a viscosity index in the range of 90 to 115 is generally preferred.

The mineral lubricating oils may be of any preferred type including those derived from the ordinary paraffinic, naphthenic, asphaltic or mixed base mineral crude oils by suitable refining methods. Synthetic hydrocarbon lubricating oils may also be employed. Other synthetic oils include dibasic acid esters such as di-2-ethyl hexyl sebacate, carbonate esters, glycol esters such as  $\text{C}_{13}$  oxo acid diesters of tetraethylene glycol, and complex esters as for example the complex ester formed by the reaction of 1 mole of sebacic acid with 2 moles of tetraethylene glycol and 2 moles of 2-ethyl hexanoic acid.

The lubricating compositions of the invention will contain between about 0.1 and 3 wt. percent, preferably from about 1 to about 2 wt. percent, of metal dialkyldithiophosphate and from about 0.05 to about 0.5 wt. percent, preferably 0.1 to 0.2 wt. percent, of the trialkylolalkane monoester. The dithiophosphates may be used without diluent or as oil solutions or concentrates containing for example 50 to 90 wt. percent metal dialkyldithiophosphate.

Antifoamants are normally not required in the lubricating oil compositions of this invention. However, a silicone fluid may be used as an antifoamant if desired. The silicone fluid, if used, will be used in concentrations ranging from 0.0001 to about 0.01 wt. percent based on the total weight of the composition. Of particular utility for obtaining additional antifoaming properties in the lubricants of this invention is Dow Corning Fluid 200.

For most applications the oxidation stability and load carrying ability imparted to the lubricating oil by the dithiophosphate additives of this invention will be entirely adequate. In some specialized applications it may be desirable to include supplemental additives. Supplemental oxidation inhibitors include the phenolic and amine inhibitors well known in the art, e.g., 2,6 di-t-butyl-p-cresol or phenyl-alpha-naphthylamine.

The nature of this invention will be more readily understood when reference is made to the accompanying examples illustrating the same.

#### EXAMPLE 1

##### *Preparation of trimethylolpropane monooleate*

The following ingredients were charged to a 4-necked distillation flask equipped with a stirrer, a thermometer, and graduated water trap with condenser:

268 grams trimethylolpropane  
566 grams oleic acid  
600 grams xylene

The reactants were heated and stirred at reflux temperature for 10 hours, with nitrogen blowing to maintain an inert atmosphere. Water and xylene were drawn off through the distillation trap throughout the course of the reaction. The following observations were made:

|                                      |           |     |
|--------------------------------------|-----------|-----|
| Initial reflux temperature           | ----- ° C | 140 |
| Final reflux temperature             | ----- ° C | 225 |
| Total water drawn off                | ----- cc  | 36  |
| Total xylene drawn off               | ----- cc  | 654 |
| Neut. Number of product (ASTM D-974) | -----     | 6.0 |

The product was then dissolved in 1000 cc. of benzene, then 500 cc. of distilled water containing 50 grams of dissolved sodium bicarbonate was added. The mixture was stirred vigorously for one hour and then allowed to separate in a 4 litre separatory funnel. Isopropyl alcohol was added until the emulsion broke and the water layer was drawn off and discarded. The neutralization number of the organic layer was 0.14. The bicarbonate wash step as above was then repeated, and the resultant organic layer was washed three times with 500 cc. portions of distilled water.

The organic layer was then vacuum stripped under a nitrogen blanket at 113° C. and 4 mm. Hg absolute pressure. The neutralization number of the final product was 1.18 and the product yield was 612 grams.

#### EXAMPLE 2

##### *Preparation of trimethylolpropane mono $\text{C}_{13}$ Oxo mercaptoacetate*

The following ingredients were charged to a 1 liter 4-necked flask equipped with a stirrer, a thermometer, and graduated water trap with condenser:

134 grams trimethylolpropane  
289 grams  $\text{C}_{13}$  Oxo mercaptoacetic acid  
300 grams xylene

The reactants were heated with stirring at reflux temperature (142-153° C.) for 4½ hours at which time 15.5 cc. of water had collected in the trap. The xylene was then stripped off under vacuum (120 mm. Hg) at a maximum temperature of 168° C. The neutralization number of the final product was 7.77 and the product yield was 397 grams.

## 5

## EXAMPLE 3

## Preparation of dialkyldithiophosphoric acid

After 450 grams of methyl isobutyl carbinol (MIBC) was heated in a reaction flask to 87° C., 245 grams of P<sub>2</sub>S<sub>5</sub> (containing 26.0% phosphorus) was added slowly over a period of 1 hour while holding the temperature at 87° C. The reaction was continued for a total time of 2½ hours. The product was then blown with nitrogen for ½ hour, cooled to 17° C., and filtered. The filtered product contained 9.28% phosphorus and 18.8% sulfur, and had a neutralization number of 184.3.

## EXAMPLE 4

## Neutralization of acid

In a reaction flask was placed 290 grams of the acid of Example 3. Then 75.4 grams of cadmium oxide was added slowly over a ½ hour period. The temperature rose to 58° C. during the addition. The temperature was further raised to 65° C. with the application of heat for a total reaction time of 3½ hours. To the reaction mixture were then added 116 grams of coastal extracted mineral oil and 12 grams of filter aid. After 10 minutes' stirring the reaction mixture was filtered through paper on a steam-heated Büchner funnel, precoated with additional filter aid. The filtrate was then dried by blowing with nitrogen under vacuum (150 mm. Hg) at 82° C. for one hour. The product was a clear, yellow, viscous liquid which, analyzed as follows:

|                       |         |       |
|-----------------------|---------|-------|
| Cadmium               | percent | 11.30 |
| Phosphorus            | do      | 6.34  |
| Sulfur                | do      | 13.10 |
| Neutralization number |         | 4.79  |

## EXAMPLE 5

Lubricating oil blends were prepared containing 1.25 wt. percent of the cadmium dialkyldithiophosphate concentrate of Example 4 and 0.035 wt. percent of an alkenyl succinic acid corrosion inhibitor obtained commercially under the trade name "Lubrizol-859." The base oil was of Mid-Continent origin, and had a viscosity of 210° F. of 59 S.S.U., a viscosity index of 105, and an API gravity of 30.2. The base oil also contained 0.0005% of a silicone anti-foaming agent (Dow Corning DC-200). To one of the blends was added 0.1 wt. percent of the additive of Example 1, to a second blend was added 0.1 wt. percent of the additive of Example 2. Each of these blends was compared in the well-known Staeger oxidation test with a third blend containing no added monoester. The results obtained are shown in Table I.

TABLE I.—STAEGER OXIDATION TEST DATA<sup>1</sup>

|                                                                                                     | Tag Robinson color after hours of test |          |          |          |
|-----------------------------------------------------------------------------------------------------|----------------------------------------|----------|----------|----------|
|                                                                                                     | Initial                                | 192 hrs. | 400 hrs. | 750 hrs. |
| Base Oil plus 1.25 wt. percent CDDP <sup>2</sup> plus 0.035 wt. percent rust inhibitor <sup>3</sup> | 18                                     | 11½      | 42       | —        |
| Blend 1 plus 0.1 wt. percent trimethylolpropane C <sub>13</sub> Oxo mercaptoacetate                 | 18                                     | 11½      | 89½      | —        |
| Blend 1 plus 0.1 wt. percent trimethylolpropane monooleate                                          | 16½                                    | 12       | 511      | 510      |

<sup>1</sup> 230° F.; Cu catalyst.<sup>2</sup> 75% concentrate of cadmium di(1,3, dimethylbutyl) dithiophosphate.<sup>3</sup> Alkenyl succinic acid rust inhibitor (16 to 18 carbon atoms in alkenyl group).<sup>4</sup> Heavy sludge.<sup>5</sup> No sludge.

As shown in the data in Table I, the blend containing only the cadmium dialkyldithiophosphate and the corrosion inhibitor was seriously degraded at the end of 400 hours and gave heavy sludge. In each case where a monoester of the present invention was also incorporated,

## 6

sludging was prevented and color degradation was markedly reduced.

## EXAMPLE 6

Blends similar to those of Example 5 were prepared using 1.5 wt. percent of the concentrate of Example 4 and the same amounts of rust inhibitor and anti-foaming agent as in Example 5. To one of these blends was added 0.2 wt. percent of trimethylolpropane monooleate and to another blend was added 0.2 wt. percent of polyethylene glycol di-tri-ricinoleate. Each of these blends, as well as a blend containing no added ester, were subjected to the Staeger oxidation test. The results are given in Table II. It will be seen that, while the trimethylolpropane monooleate of the present invention prevented degradation of the oil in much the same manner as in Example 5, the polyethylene glycol ester was not nearly as effective in preventing degradation.

TABLE II.—STAEGER OXIDATION TEST

[230° F.—copper catalyst]

|                                                                                                                                                                          | Tag-Robinson color after hours of test |           |           |
|--------------------------------------------------------------------------------------------------------------------------------------------------------------------------|----------------------------------------|-----------|-----------|
|                                                                                                                                                                          | Initial                                | 192 hours | 400 hours |
| 25                                                                                                                                                                       |                                        |           |           |
| (1) Base oil plus 1.5 wt. percent CDDP <sup>a</sup> plus 0.035 wt. percent rust inhibitor <sup>b</sup>                                                                   | 13½                                    | 9½        | 2         |
| (2) Blend 1 plus 0.2 wt. percent trimethylolpropane monooleate                                                                                                           | 13½                                    | 10½       | 10        |
| (3) Blend 1 plus 0.2 wt. percent ethylene glycol di-tri-ricinoleate                                                                                                      | 13½                                    | 10        | 4½        |
| (4) Base oil <sup>c</sup> plus 1.5 wt. percent CDDP plus 0.035 wt. percent rust inhibitor <sup>b</sup> plus 0.2 wt. percent trimethylolpropane monostearate <sup>d</sup> | 15                                     | 11½       | 9½        |
| 30                                                                                                                                                                       |                                        |           |           |
| 35                                                                                                                                                                       |                                        |           |           |

<sup>a</sup> 75% concentrate of cadmium di(1,3, dimethylbutyl) dithiophosphate.<sup>b</sup> Alkenyl succinic acid rust inhibitor (16 to 18 carbon atoms in alkenyl group).<sup>c</sup> Difference in initial color is due to different sample of the base stock, which otherwise duplicated the base stock of Blend 1.<sup>d</sup> Prepared in a manner similar to that for preparation of trimethylolpropane monooleate as in Example 1.

Blend 2 of Table II gave a rating of 98 in the IAE Gear Test, thus meeting the 90 minimum requirement of both the British and Canadian Navies. It also passed 12 load stages with no extreme wear in the FZG Niemann Gear Test.

It is to be understood that the examples presented herein are intended to be merely illustrative of the invention and not as limiting it in any manner; nor is the invention to be limited by any theory regarding its operability. The scope of the invention is to be determined by the appended claims.

## What is claimed is:

1. An improved marine turbine oil composition comprising a major proportion of a lubricating oil, from about 1 to about 3 wt. percent of an oil soluble cadmium salt of a dialkyldithiophosphoric acid having alkyl groups derived from secondary alcohols and containing from about 3 to about 20 carbon atoms per alkyl group with an average of at least 4.5 carbon atoms per alkyl group, and from about 0.05 to about 0.5 wt. percent of a monoester of a neo-structured trialkylolalkane of from 6 to 12 carbon atoms and of a carboxylic acid selected from the group consisting of saturated and unsaturated fatty acids of from 12 to 20 carbon atoms and alkyl mercaptoacetic acids having alkyl groups of from 9 to 18 carbon atoms.

2. Composition as defined by claim 1 wherein said monoester is trimethylolpropane monooleate.

3. Composition as defined by claim 1 wherein said monoester is trimethylolpropane monostearate.

4. Composition as defined by claim 1 wherein said monoester is trimethylolpropane C<sub>13</sub> oxo mercaptoacetate.

5. Composition as defined by claim 1 including from 0.005 to 0.5 weight percent of a corrosion inhibitor selected from the group consisting of alkyl mercaptoacetic

acids having alkyl groups of from 9 to 18 carbon atoms and alkenyl succinic acids having from 10 to 20 carbon atoms in the alkenyl group.

**References Cited by the Examiner**

| UNITED STATES PATENTS |      |               |            |
|-----------------------|------|---------------|------------|
| 2,371,333             | 3/45 | Johnston      | 252—48.6   |
| 2,477,356             | 7/49 | Wayo          | 252—48.6   |
| 2,560,202             | 7/51 | Zimmer et al. | 252—33.4   |
| 2,601,063             | 6/52 | Smith et al.  | 252—48.6 X |

5.

|           |       |               |            |
|-----------|-------|---------------|------------|
| 2,603,653 | 7/52  | Kosmin et al. | 252—48.6 X |
| 2,884,379 | 4/59  | Rudel et al.  | 252—48.6   |
| 2,911,367 | 11/59 | Baus et al.   | 252—32.7   |
| 3,013,971 | 12/61 | Mastin        | 252—32.7   |

FOREIGN PATENTS

|         |      |         |
|---------|------|---------|
| 536,837 | 2/57 | Canada. |
|---------|------|---------|

DANIEL E. WYMAN, Primary Examiner.

10. JOSEPH R. LIBERMAN, Examiner.